

Jan. 16, 1940.

I. V. MANSELL

2,186,982

SIGN

Filed Jan. 11, 1938



Fig. 1



Fig. 4



Fig. 5



Fig. 3



Fig. 6



Fig. 7

INVENTOR  
Irving V. Mansell  
BY  
Grooster & Davis  
ATTORNEYS.

## UNITED STATES PATENT OFFICE

2,186,982

## SIGN

Irving V. Mansell, Bridgeport, Conn.

Application January 11, 1938, Serial No. 184,442

17 Claims. (Cl. 40—130)

This invention relates to display signs and the like, and particularly to an improved face plate for such signs or displays or surface finishes where the hard glossy surface finish of glass is an advantage.

It is an object of the invention to provide a glass face structure which is especially adapted for use with elongated tubular lamp signs and which adds to such signs shatter-proof or safety characteristics, permitting the use of ordinary glass for the face of the sign and also to add additional strength to such ordinary glass and permits greater deflection thereof under nominal pressures without cracking or breaking of the glass.

It is also an object of the invention to provide a composite glass face section which can be readily made translucent, transparent or opaque as desired, to most effectively bring out the display matter. Also to make a construction wherein the back or rear side of the face of the sign display forms an admirable base for the mounting of the tubular lamps with the necessary appurtenances inside the sign.

It is a further object of the invention to provide a construction which will seal in on the face of the glass in a substantially permanent manner the various colors and designs required for any particular sign or display, and also to provide a construction which affords protection for the various colors from deterioration because they are sealed in and bonded to the glass.

Still another object of the invention is to provide a construction which has heat insulating properties so that comparatively hot tubular lamps may be placed immediately on the back of the composite glass faces with a minimum of danger of the heat cracking or breaking the glass.

A still further object is to provide a construction in which the composite background which is bonded to the glass face can be readily bonded or adhered to any other solid, hard, stiff, or pliable material where the surface effect of the glass is desired, such for example as in store fronts and other surfaces of veneer finish.

With the foregoing and other objects in view which will become apparent as the description proceeds, I have devised a construction, certain embodiments of which are illustrated in the accompanying drawing forming a part of this specification. It is, however, to be understood that various changes and modifications may be employed within the scope of the invention. Also, the invention is not confined to the use of glass

but other plastics which have been used as glass substitutes may be employed.

In this drawing:

Fig. 1 is a front face view of the upper portion of a sign embodying this invention;

Fig. 2 is a vertical transverse section thereof on an enlarged scale;

Fig. 3 is a rear view of one of the characters in the sign of Figs. 1 and 2;

Fig. 4 is a detailed section of a portion of a face plate which may be used for such sign;

Fig. 5 is a similar view showing a somewhat different construction which may be used for larger face plates;

Fig. 6 is a detailed section taken substantially on line 6—6 of Fig. 3 showing the use of the construction of Fig. 4; and

Fig. 7 is a similar section showing the use of the construction of Fig. 5.

The sign construction shown in Figs. 1 and 2 is a double faced sign comprising the two opposite faces 10 and 11 held at the desired distance apart by any suitable mounting or frame construction. In the present case, by way of example, these two faces are mounted in a circular metal frame 12 having inwardly extending flanges 13 behind which the faces 10 and 11 are mounted.

Between these two face plates 10 and 11 are mounted the illuminated lamps indicated in the present instance as elongated luminous tubes 14. These may be of any suitable lamp construction, a common lamp in use at the present time being the so-called "neon" or luminous glass tube lamps. These lamps are generally called "neon" or "neon type" lamps although they may be filled with different gases than neon gas, such for example as helium, argon, or the like or mixtures of the same. Other tubular lamps such as filament lamps may also be used.

As this is a double faced sign and the display characters on the two faces 10 and 11 may be different or reversed, there is shown in the drawing two of these luminous tubes or lamps, one immediately behind each face plate to illuminate the display matter thereon. In the present case there is shown a partition 15 between the lamps and cross baffles 16 extending across the space between the face plates and the partition to confine and diffuse the light, these baffles being mounted in any suitable manner, as for example by small brackets 17 cemented to the baffles 16 and the backing on the plates, but it is to be understood this construction and arrangement is shown merely by way of example and that any desired construction and arrangement may be employed.

5

15

20

25

30

35

40

45

50

55

The faces 10 and 11 are of improved construction which gives the required strength and desirable non-shatterable properties without the use of objectionably thick and heavy glass plates. 5 Two specific constructions involving this new principle are shown in detail in Figs. 4 and 5. In Fig. 4 there is shown a glass plate 20 mounted on the rear face of which is a fibrous reenforcing sheet 21, this sheet being securely bonded to the 10 rear face of the glass 20 by a layer 22 of non-shattering adhesive resin. In the form shown in Fig. 5 the strength of the fibrous sheet 21 is still further increased by a fabric sheet 23 thoroughly bonded with the fibrous sheet 21, and this 15 composite sheet is bonded to the rear face of the glass by the layer of non-shattering adhesive resin 22 the same as in the form of Fig. 4. It will be evident that the construction of Fig. 4 does not have the additional strength and resistance to 20 breaking which the form of Fig. 5 has but may be sufficient for smaller signs, while the construction of Fig. 5 has sufficient strength for any of the larger signs now at present employed.

There are a number of materials which may 25 be used for these reenforcing backing sheets 21, the preferred being a sheet of asbestos fiber as this is fireproof and has other desirable characteristics, but there are other materials which may be used in place of the asbestos, such for example as 30 canvas, duck, heavy paper, Bakelite and a number of other materials, depending upon the purpose to which the invention is put. Similarly the reenforcing woven fabric sheet 23 may be of different materials, such for example as 35 canvas pasting material, cheesecloth, and other fabrics. As indicated, however, I have found that for the backing up material sheet asbestos alone is very satisfactory for the small areas, while this sheet asbestos with the bonded inner 40 layer of fabric 23 to add strength is preferred for the larger areas and for outside signs where additional strength and safety qualities are desired. This composite backing 21 and 23 may be made by laying together the layer of asbestos 45 fiber and the woven cloth fabric while the asbestos is still moist and pressing them firmly together by running them through rolls. This provides a substantially unitary structure which is very effective in combination with the layer of adhesive resin in imparting to the glass the desired 50 strength and non-shatterable qualities.

The non-shatterable adhesive material 22 may be any of a number of different materials of resin or cellulose material some of which are now 55 commonly employed in making laminated, non-shatterable glass for use in automobiles, and these materials may be purchased on the market under various names. I prefer for sign and display work a suitable adhesive such as is provided 60 in the acrylic and methacrylate resins. In making up these improved face plates I take a sheet of glass 20 as thin as practical for the desired area and coat one side of this glass sheet with a suitable adhesive such for example as the acrylic or methacrylate resins in a suitable solvent, and 65 before this is applied to the glass there may be thoroughly mixed with it the required color in dye, pigment, or other coloring matter, desired for the display matter. A layer of this same adhesive resin is also applied to or incorporated in the fibrous sheet or backing 21, or the composite sheet 21, 23 depending on which is used, which 70 layer of resin also partially saturates this fibrous sheet, and this resin coating as applied to the fibrous sheet also has incorporated in it the same

color as is in the layer applied to the glass sheet. These prepared sheets of glass and fibrous material are then suitably processed or bonded to each other to make one composite face.

The display or character strokes as required 5 for the display matter, such as those indicated for example at 24, are then outlined and cut or otherwise imposed upon or through the layers of fibrous material and resinous material, so that this asbestos or fibrous material and other coatings within the cutlines of the character strokes may be removed from the back of the glass sheet, exposing clear glass between these areas. The clear glass character strokes are generally coated on the clear glass within the cut out sections with 10 a similar resinous material as indicated at 22a to which has been added the desired color, or if a clear stroke is desired no color at all, so that the face of the display will present the required 15 design and color effects when viewed from the front. This replacement coating 22a within the outline of the character strokes being of the same base material as the adhesive resin which immediately bonds with said resinous material between the fibrous sheet and the glass thereby creates the effect of carrying shatter-proof qualities 20 across said character strokes providing a degree of replacement for the fibrous or asbestos sheet and resin layers which have been removed.

Another method by which this composite sign 30 face with the character strokes showing thereon may be produced is to cut out the character strokes in the required design in the asbestos or fiber sheet before the application of the resin and the bonding of the fibrous reenforcing sheet 35 to the glass sheet. Also, other methods or processes for obtaining the same result will be apparent and will be developed in practice.

It has been found in practice that the combination of this reenforcing or fibrous layer 21 or 40 21-23 with the layer of non-shattering adhesive in bonding these fibrous materials to the glass makes a much stronger construction and one which will be much less liable to shatter than are 45 constructions using the non-shattering adhesive resin alone, permitting the use of much thinner and therefore lighter glass sheets, which is very important in glass display signs which must be suspended outdoors or over areas which are used for passage by individuals such for example as 50 sidewalks and similar areas. I have also found that this combination permits the glass to yield or flex further under a blow or lateral pressure before the glass will crack.

It will be evident from the foregoing description 55 that it provides a composite glass plate which can be readily made translucent, transparent or opaque. The fibrous back also makes an admirable medium or base for the mounting of the tubular lamps or other necessary appurtenances within the sign, as the required mounting elements may be readily secured to this fibrous back by various adhesives, which much more readily adhere to this material than they would to the face of the glass plate itself and as well 60 avoid the possibility of causing a mark on the face of the display opposite the mounting. It will also be apparent that in this construction the pigment or coloring matter is sealed on to the glass face in 65 a substantially permanent manner, because it is incorporated in the layer of adhesive resin which is between the fibrous sheet and the glass. This also affords protection for these various colors from deterioration so that the display sign mat- 70 75

ter retains its true colors and brilliancy more permanently.

This composite construction involving the asbestos or other fibrous layer and the layer of adhesive resin still further provides a very effective insulation for heat or cold so that comparatively hot tubular lamps may be placed immediately on the back of the sheets or composite faces, without danger of the heat of the lamp cracking or breaking the glass, and if the fibrous material is of asbestos it also has the effect of rendering the adhesive resin layer non-inflammable. Still further due to the fact that this fibrous layer may be readily bonded to other materials and much more readily than glass could be, this composite glass sheet may be used for store fronts and other similar uses where the mounting requires adhering to other solid, hard, stiff or pliable material and where it is desirable to have the lustrous finish of a glass for the exterior surface.

It is to be understood that the term "glass sheet" is used in the broad sense to include other plastics which are in some cases being used as glass substitutes.

Having thus set forth the nature of my invention, what I claim is:

1. A non-shatterable glass face for a sign or the like comprising a sheet of glass to one face of which is secured a fibrous reenforcing sheet by an intermediate layer of non-shatterable adhesive.

2. A glass face for a sign or the like comprising a sheet of glass, a sheet of fibrous material including a sheet of asbestos fibre and a sheet of fabric bonded therewith, and said sheet of fibrous material being secured to a face of the glass by an intermediate layer of non-shatterable adhesive.

3. A non-shatterable glass face for a sign or the like comprising a sheet of glass, a sheet of fibrous reenforcing material including a woven fabric, and said sheet of fibrous material being secured to one face of the glass by an intermediate layer of a non-shatterable adhesive.

4. A non-shatterable glass face for a sign or the like comprising a sheet of glass, a sheet of fibrous reenforcing material, said sheet of fibrous material being secured to a face of the glass by an intermediate layer of a non-shatterable adhesive, and a colored pigment or dye incorporated in said adhesive.

5. A glass face for a sign or the like comprising a sheet of glass, a reenforcing fibrous sheet including a sheet of asbestos fibre and a sheet of fabric bonded therewith, said fibrous sheet being secured to a face of the glass by a layer of non-shatterable adhesive, and colored pigment or dye incorporated in said adhesive.

6. A glass face for a sign comprising a sheet of glass, a reenforcing sheet of fibrous material secured to a face of the glass by a layer of non-shatterable adhesive, said fibrous sheet being cut away to permit passage of light and form character strokes, and the surface of the glass in said strokes being covered with said adhesive.

7. A sign comprising a face including a glass sheet, a reenforcing fibrous sheet on the rear face of said glass including asbestos fibre, said fibrous sheet being secured to the face of the glass by a layer of non-shatterable adhesive, portions of said fibrous sheet being cut out to form character strokes, and an elongated tube lamp at the rear of said fibrous sheet to illuminate said strokes.

8. A display sign comprising a glass sheet, a reenforcing fibrous sheet at the rear of said glass

including a sheet of asbestos fibre and a strengthening fabric bonded therewith, said fibrous sheet being secured to the face of the glass by a layer of non-shatterable adhesive, said fibrous sheet having portions cut out to provide character strokes, the glass surface in said strokes being covered with said adhesive, and an elongated tube lamp at the rear of said fibrous sheet to illuminate said strokes.

9. A display sign comprising a glass sheet, a reenforcing fibrous sheet at the rear face of said glass, said fibrous sheet being secured to the face of the glass by a layer of non-shatterable adhesive, portions of said fibrous sheet being cut away to form character strokes, colored pigment or dye incorporated in said adhesive layer to form a background for the character strokes, and an elongated tube lamp at the rear of the fibrous sheet to illuminate said character strokes.

10. A display sign comprising a glass sheet, a reenforcing fibrous sheet at the rear of said glass, said fibrous sheet being secured to the inner face of the glass sheet by a layer of non-shatterable adhesive, said fibrous sheet and layer of adhesive having portions cut out to provide character strokes, the glass surface in said strokes being covered with similar adhesive, said adhesive having color incorporated as required for color of character strokes contrasting with the background for daylight visibility, and an elongated tube lamp at the rear of the fibrous sheet to illuminate said character strokes.

11. A display finish for store fronts and the like comprising a sheet of glass, a sheet of reenforcing fibre at the rear of said glass bonded therewith, said fibrous sheet being secured to the face of the glass by a layer of non-shatterable adhesive, colored pigment, dye or other coloring material being incorporated in the adhesive to form the color required for the surface finish.

12. A preformed shatter-proof or safety structural unit comprising a sheet of glass to one face of which is secured a fibrous reenforcing sheet by an intermediate layer of non-shatterable adhesive.

13. A non-shatterable glass face of composite structure, comprising a sheet of glass for the surface sheet, said glass sheet being backed up by a reenforcing sheet of fibrous material, said two sheets being bonded into one unit composite face by an intermediate layer of non-shatterable adhesive, and desired coloring to show from the front through the glass being incorporated in or between the two sheets.

14. A non-shatterable glass face of composite structure comprising a sheet of glass for the surface sheet, said glass sheet being backed up by a reenforcing sheet of fibrous material, said two sheets being bonded together into one unit composite face by an intermediate layer of non-shatterable adhesive.

15. A non-shatterable glass face of composite structure comprising a sheet of glass for the surface sheet, said glass sheet being backed up by a reenforcing sheet of woven fabric, said two sheets being bonded together into one unit composite face by an intermediate layer of non-shatterable adhesive.

16. A non-shatterable glass face of composite structure, comprising a sheet of glass for the surface sheet, said glass sheet being backed up by a reenforcing sheet of fibrous material, said two sheets being bonded into one unit composite face by an intermediate layer of non-shatterable adhesive, and desired coloring either as plain back-

ground or background with character strokes or designs to show from the front through the glass being incorporated in or between the two sheets.

17. A non-shatterable glass face of composite structure, comprising a sheet of glass for the surface sheet, a sheet of fibrous material including

an unwoven fibrous sheet and a sheet of woven fabric bonded therewith, and said sheet of fibrous material being secured to the rear face of said glass by an intermediate layer of non-shatterable adhesive.

IRVING V. MANSELL. 5